

Dec. 29, 1953

P. R. HINES  
DIFFERENTIAL FROTH FLOTATION PROCESS

2,664,198

Filed Dec. 26, 1950

3 Sheets-Sheet 1



Fig. 1

INVENTOR.  
Pierre R. Hines

BY

*Roger S. Sernoff*

ATTORNEY

Dec. 29, 1953

P. R. HINES

2,664,198

DIFFERENTIAL FROTH FLOTATION PROCESS

Filed Dec. 26, 1950

3 Sheets-Sheet 2



INVENTOR.  
Pierre R. Hines

BY  
Robert W. Rosenoff

ATTORNEY

Dec. 29, 1953

P. R. HINES

2,664,198

DIFFERENTIAL FROTH FLOTATION PROCESS

Filed Dec. 26, 1950

3 Sheets-Sheet 3



Fig. 3

INVENTOR.  
Pierre R. Hines

BY  
Leona S. Banoff

ATTORNEY

## UNITED STATES PATENT OFFICE

2,664,198

DIFFERENTIAL FROTH FLOTATION  
PROCESS

Pierre R. Hines, Portland, Oreg.

Application December 26, 1950, Serial No. 202,643

4 Claims. (Cl. 209—167)

1

This invention relates, broadly, to the separation of minerals and the concentration of ores by froth flotation; more particularly, it relates to the separation of lead and zinc from an ore containing these.

This invention is based upon the discovery that urea and its derivatives are effective flotation agents and can be used advantageously as mineral collecting agents in froth flotation operations. These compounds are highly selective towards a single metal radical and when used in a circuit of controlled alkalinity and give improved results in the differential flotation of complex lead-zinc ores. They can be used to advantage in flotation operations on lead-zinc ores under controlled conditions of alkalinity because they do not require the various supplementary reagents such as conditioners and depressers or, if these are required, a smaller quantity can be employed.

In addition, urea and its derivatives are of lower unit cost than the reagents used heretofore so that the overall reagent cost per ton of ore treated is materially reduced. Further, urea and its derivatives are more selective in their action, particularly on lead-zinc ores, than the agents known heretofore.

The compounds which can be employed are represented by the formula:



These compounds, R<sub>1</sub>, R<sub>2</sub>, R<sub>3</sub>, and R<sub>4</sub>, are hydrogen, an aliphatic or an aromatic group; more particularly, one can employ as typical aliphatic group an alkylene group such as allyl or an alkyl group, the methyl, ethyl, butyl, propyl, hexyl, etc.; as an aromatic, one can use any aryl substituent, but the cheapest and most common is the phenyl group. Generally, the more carbon atoms included in the compound, the greater is the collecting power. In the above formula, the substitution for hydrogen can be made with any number of substituents, that is, one, two, three or four, and the substituents can be different in the several positions, that is, the compound can include the same group in two or more positions as diphenyl urea, or two or more different groups as ethyl phenyl urea and ethyl diphenyl urea.

The value and practice of the invention will become further apparent after consideration of the following specific examples which are set forth by way of illustration. The test material employed was a typical sample of the mill feed at

2

the Bunker Hill & Sullivan Mining & Concentrating Co., at Kellogg, Idaho, and composed of one third mine ore and two thirds old jig tailings.

The zinc sulphide in the Bunker Hill & Sullivan ores occurs as several varieties of sphalerite, e. g., a light-colored sphalerite which is very difficult to depress, followed by darker shades and a black zinc sulphide, said to be marmatite, a ferri-ferrous variety containing 10% or more of iron. High zinc losses are frequently attributed to the presence of marmatite and the difficulty in float-  
10 ing it. The ore is inherently difficult to treat for zinc and consequently the recovery of zinc in the zinc concentrate is low. The present standard practice on this ore includes grinding of the feed to a fineness of 62% minus 200 mesh and the addition of the following reagents to the ball mill:

|                             | Pounds per ton of ore |
|-----------------------------|-----------------------|
| Soda Ash                    | 1.1                   |
| Sodium cyanide              | 0.15                  |
| Zinc sulphate               | 0.40                  |
| Potassium ethyl xanthate Z3 | 0.015-0.03            |
| Frother                     | 0.1-0.2               |

20 The frother employed was a mixture of 5% amyl alcohol, 10% pine oil and 85% Barrett's No. 4 coal tar creosote. The pH of the lead section was 7.1 and that of the zinc section 7.2.

Reagents added to zinc section:

|                             | Pounds     |
|-----------------------------|------------|
| Lime                        | 0.3        |
| Copper sulphate             | 0.33       |
| Potassium ethyl xanthate Z3 | 0.015-0.03 |
| Frother                     | 0.05-0.1   |

30 The flotation process consists of a rougher step followed by three cleaning steps upon both the lead and zinc section, to produce the final grades of lead and zinc concentrate.

40 A typical monthly average of the metallurgical results obtained by the described mill practice upon this feed is given below:

|                  | Feed    |         | Recoveries |         |
|------------------|---------|---------|------------|---------|
|                  | Lead    | Zinc    | Lead       | Zinc    |
| Mill feed        | Percent | Percent | Percent    | Percent |
| Lead concentrate | 4.83    | 1.35    | 100        | 100     |
| Zinc concentrate | 70.09   | 5.01    | 91.73      | 23.48   |
| Tail             | 3.23    | 53.14   | 0.94       | 55.38   |
|                  | 0.38    | 0.31    | 7.33       | 21.14   |

45 In the tests conducted to illustrate this invention and reported here as Examples 1, 2 and 3, the feed sample utilized contained 4.52% lead

and 1.08% zinc. The feed sample was ground wet in a steel rod mill to 62% minus 200 mesh, the flotation reagents for the lead flotation being added to the rod mill. The pulp was then transferred to a GECO flotation cell which utilizes a combination of mechanical and pneumatic agitation. The oil mixture frother given above was used, but no other flotation reagent or depressing agent was employed. The pulp was subjected to agitation and aeration and the lead froth concentrate removed. The reagents for zinc flotation were then added to the flotation cell and the pulp again subjected to agitation and aeration and the zinc froth concentrate removed. Comparisons were made between the various flotation reagents contemplated by this invention with potassium ethyl xanthate following the previously described mill practice on this ore feed. The results, shown graphically in Figures 1, 2 and 3, are entirely from rougher concentrates with no cleaning steps.

Referring to the drawings, Figure 1 illustrates graphically the lead recovery with 0.1 lb. of urea per ton of ore while the amount of sodium carbonate was varied from 0.3 lb. per ton to 4 lb. per ton; also shown is the percentage of the total zinc which floated with the lead concentrate, as is the grade of the lead concentrate, i. e., the percentage of lead in the lead concentrate.

In Figure 2 are shown graphically the results obtained on this ore when the quantity of urea was varied from 0.03 lb. per ton to 0.4 lb., the sodium carbonate being held at a constant quantity of two pounds per ton, the per cent of the total zinc floating with the lead concentrate, and the grade of the lead concentrate.

In Figure 3 are shown graphically the results when the quantity of urea was varied and the sodium carbonate was held constant at 3 lb. per ton.

A study of these graphical showings will reveal that the lead recovery rises rapidly until 2 pounds of sodium carbonate is reached, a pH of approximately 8.0 for this ore. As the amount of sodium carbonate is increased beyond 2 pounds per ton, the lead recovery rises very slowly.

In the Bunker Hill & Sullivan ore, the lead-zinc ratio is high, about 4.5 to 1, while the zinc content in the feed is lower than in most lead zinc mill tails. If more zinc is depressed by using depressing agents such as zinc sulphate or cyanide the recovery of lead is lowered. The total economic recovery of both lead and zinc determines the lead recovery and the corresponding percentage of the zinc in the lead concentrate.

#### EXAMPLE I

Table 1

| Collector      | Sodium carbonate, lb. | Percent lead recovery | Percent total zinc in lead concentrate | Percent lead in lead concentrate |
|----------------|-----------------------|-----------------------|----------------------------------------|----------------------------------|
| Z-3*, 0.06 lb. | 1.1                   | 92.9                  | 56.4                                   | 54.7                             |
| Urea, 0.1 lb.  | 3.0                   | 92.6                  | 54.7                                   | 53.6                             |
| Do.            | 2.0                   | 92.8                  | 55.1                                   | 53.4                             |

\*Z-3—potassium ethyl xanthate, fed with 0.15 lb. per ton of sodium cyanide and 0.40 lb. of zinc sulfate. (Z is the registered trade-mark of The Dow Chemical Company for its xanthate flotation reagents.)

A study of the results shown in Figures 1, 2 and 3 with the comparative results in Table 1 above show that the same results can be obtained with urea alone as with potassium ethyl xanthate and zinc sulphate and sodium cyanide as depressing agents.

The percentage of the total zinc floating with the lead concentrate rises rapidly when the quantity of sodium carbonate is increased beyond 3 pounds per ton, which corresponds to a pH of approximately 8.6. The upper critical point for the Bunker Hill & Sullivan ore is determined by the best economic recovery of both lead and zinc rather than the higher lead recoveries with greater amounts of sodium carbonate and a higher pH. Similar values may be ascertained for other lead-zinc ores by test and the best economic recovery determined.

Urea has the advantage of being only approximately one-third the cost per pound of potassium ethyl xanthate; further, it does not require depressing agents to secure the same results, giving definite savings in reagent cost. It is a simple problem to control the amount of urea and the amount of sodium carbonate fed as these can be added automatically; it has been demonstrated that automatic feed of flotation reagents give improved operating results as compared to depending upon the operator's judgment as to the amounts to be fed.

#### EXAMPLE II

In Table 2 below, I have shown the results on this same ore with urea, the alkyl and aryl ureas, without the use of depressing agents, as well as the results with urea, the alkyl ureas, aryl ureas, and potassium ethyl xanthate using depressing agents for the zinc. Referring to Table 2, tests 4-9 show clearly the gradually increasing collecting power of the alkyl and aryl ureas as the number of carbon atoms increases; these also show the increase in the quantity of zinc which floats with the lead in this ore when no depressing agent is used.

Table 2

(\* See notes below.)

| Test | Collector                | Sodium carbonate | Lead, percent recovery | Percent total zinc in lead concentrate | Grade lead concentrate, percent lead |
|------|--------------------------|------------------|------------------------|----------------------------------------|--------------------------------------|
| 1    | 0.1 lb. urea             | 2.0              | 92.8                   | 55.1                                   | 53.4                                 |
| 2    | do                       | 3.0              | 92.6                   | 54.7                                   | 53.6                                 |
| 3    | 0.2 lb. urea             | 2.0              | 91.7                   | 47.1                                   | 56.0                                 |
| 4    | 0.2 lb. monoethyl urea   | 2.0              | 89.9                   | 50.1                                   | 58.6                                 |
| 5    | 0.1 lb. S-Di-n-butylurea | 1.0              | 93.1                   | 67.3                                   | 59.2                                 |
| 6    | do                       | 3.0              | 96.5                   | 73.9                                   | 47.9                                 |
| 7    | 0.1 lb. phenyl urea      | 3.0              | 96.1                   | 67.1                                   | 51.6                                 |
| 8    | do                       | 4.0              | 95.6                   | 59.4                                   | 52.0                                 |
| 9    | 0.1 lb. di-phenyl urea   | 3.0              | 94.5                   | 67.2                                   | 54.8                                 |
| 10*  | 0.06 lb. Z-3             | 1.1              | 92.9                   | 56.4                                   | 54.7                                 |
| 11*  | 0.1 lb. urea             | 4.0              | 93.3                   | 54.3                                   | 53.7                                 |
| 12*  | 0.2 lb. urea             | 2.0              | 90.4                   | 35.0                                   | 57.8                                 |
| 13*  | do                       | 2.0              | 91.4                   | 51.7                                   | 56.4                                 |
| 14*  | do                       | 2.0              | 88.9                   | 49.8                                   | 57.3                                 |
| 15*  | do                       | 2.0              | 91.8                   | 58.4                                   | 57.5                                 |
| 16*  | do                       | 2.0              | 87.6                   | 41.5                                   | 60.4                                 |
| 17*  | 0.1 lb. S-Di-n-butylurea | 3.0              | 93.3                   | 64.3                                   | 57.3                                 |
| 18*  | do                       | 3.0              | 93.3                   | 64.3                                   | 57.3                                 |

10\* and 11\*—fed with 0.15 lb. per ton of sodium cyanide and 0.4 lb. per ton of zinc sulfate.

12\* and 17\*—fed with 0.8 lb. per ton of zinc sulfate.

13\*—fed with 0.4 lb. per ton of zinc sulfate.

14\*—fed with 0.1 lb. per ton of sodium sulfate.

15\*—fed with 0.3 lb. per ton of sodium cyanide.

16\* and 18\*—fed with 1.0 lb. per ton of sodium hydroxide.

The standard comparison test for potassium ethyl xanthate using depressing agents is given in Test 10. Tests 11-18 above show results when depressing agents are used with urea, the alkyl and aryl ureas; while depressing agents may be used in conjunction with urea, alkyl ureas and aryl ureas, they are not essential.

A study of Table 2 will also bring out clearly the advantages of urea and its derivatives as

collectors for lead. The results show an increase in collecting power affects both the lead and zinc in the absence of a zinc depressant. If a zinc depressant is employed to suppress the zinc while floating the lead, some lead recovery is sacrificed to achieve any substantial depression of the zinc as compared to urea alone. While these results apply specifically to the Bunker Hill and Sullivan ore treated, the selection and choice of reagents on an ore is determined by the best economic recovery rather than the best metallurgical recovery; the results in this table show the wide field of choice possible with urea and its derivatives.

EXAMPLE III

Zinc sulphide requires a powerful collector and activation with copper sulphate for successful flotation by either potassium ethyl xanthate or urea or its derivatives. In Table 3 I have set forth the results on the test ore using 0.33 lb. per ton of copper sulfate to establish a comparison between potassium ethyl xanthate following standard mill practice for the Bunker Hill & Sullivan ore and the derivatives of urea. It is to be noted that the use of S-Di-n-butylurea cut the loss of zinc in the tails approximately in half and at the same time doubled approximately the grade of the concentrate.

Table 3

| Test | Collector                                     | Lime, lbs. per ton | Percent zinc in tails | Percent of total zinc loss in tails | Grade of zinc concentrate |
|------|-----------------------------------------------|--------------------|-----------------------|-------------------------------------|---------------------------|
| 1    | 0.06 lb. Z-3                                  | 0.3                | 0.22                  | 17.6                                | 13.7                      |
| 2    | 0.1 lb. phenyl urea                           | 1.5                | 0.18                  | 15.9                                | 19.1                      |
| 3    | 0.1 lb. diphenyl urea                         | 1.5                | 0.15                  | 12.5                                | 20.6                      |
| 4    | 0.1 lb. ouramine (70% n-butyl urea-30% urea). | 1.0                | 0.12                  | 10.8                                | 9.8                       |
| 5    | 0.1 lb. S-Di-n-butylurea                      | 1.0                | 0.10                  | 8.7                                 | 17.1                      |
| 6    | do                                            | 2.0                | 0.10                  | 8.9                                 | 25.2                      |
| 7    | do                                            | 3.0                | 0.13                  | 11.2                                | 24.6                      |

When depressing agents are used in the lead section for suppressing the flotation of the zinc with the lead concentrate, it is necessary to increase the lime to at least three pounds per ton, corresponding to a pH of approximately 9.2. The preceding lead float may employ potassium ethyl xanthate as a collector as well as urea and its derivatives without affecting the zinc float except when used in conjunction with depressing agents mentioned before. The black sphalerite is seen in the tails under a microscope when the tails are high. They are absent when the tails are low. When the tails are low, the concentrate assumes a salt and pepper appearance to the naked eye and, under the microscope, the black sphalerite can be clearly identified. It is probable the superior recovery is due to an improved collecting power for the more difficult varieties of sphalerite in this ore.

The pH on the Bunker Hill & Sullivan ore for the corresponding amounts of lime is given below:

|     | pH | Pounds of lime per ton |
|-----|----|------------------------|
| 8.2 |    | 1.0                    |
| 8.7 |    | 2.0                    |
| 9.2 |    | 3.0                    |

The concentrate grade is higher with the higher pH and, as the urea derivatives give better results with a higher lime, the depression of the pyrite is better. It will be noted in Table 3

that the standard mill practice requires 0.3 lb. lime with a pH of 7.2, which is not favorable for depressing pyrite.

The several examples given above show the general characteristics of urea and its derivatives as collectors for lead and zinc minerals. Tests with pure minerals show urea has very little selective action towards pyrite. Due to the good collecting action of the urea derivatives with a high pH and with lime, good depression of pyrite is secured, and pyrite is plainly identifiable under the microscope when the zinc concentrate grade is high, as is shown by Example III.

Urea is water soluble as are methyl, ethyl, butyl and diethyl urea; dibutyl urea, phenyl and diphenyl ureas are only slightly soluble in water, but all are soluble in methyl alcohol and can be fed in solution. Those which are insoluble or only slightly soluble are miscible with water and can be fed dry to the rod mill preceding the lead float and with the copper sulphate preceding the zinc float.

Urea is used in large quantities for a number of purposes in the chemical industry and is readily procurable from a number of chemical manufacturers. As a collector, its price is about a third approximately of other collectors on the market. The commercial manufacture of the alkyl and aryl ureas has, in most cases, been worked out, and several are on the market. The characteristics are shown so that any one versed in the flotation art may in the usual manner by tests apply urea and its derivatives to a lead-zinc ore flotation problem.

I claim:

1. A method of differential froth flotation which comprises subjecting an aqueous alkaline pulp of an ore containing lead and zinc to froth flotation in the presence of a frother and in the presence of a reagent included in the group having the following formula:



where  $R_1$  and  $R_3$  are hydrogen atoms and  $R_2$  and  $R_4$  are members chosen from the group including hydrogen, aliphatic radicals and aromatic radicals, and removing therefrom a concentrate containing lead and a tailing rich in zinc.

2. A method of differential froth flotation which comprises subjecting an aqueous alkaline pulp of an ore containing lead and zinc to froth flotation in the presence of a frother and in the presence of a reagent included in the group having the following formula:



where  $R_1$  and  $R_3$  are hydrogen atoms and  $R_2$  and  $R_4$  are members chosen from the group including hydrogen, aliphatic radicals and aromatic radicals, removing therefrom a concentrate containing lead and a tailing rich in zinc, activating the zinc with copper sulfate subjecting an aqueous alkaline pulp of the tailing to froth flotation in the presence of a reagent included in the group having the following formula:



where  $R_1$  and  $R_3$  are hydrogen atoms and  $R_2$  and  $R_4$  are members chosen from the group including hydrogen, aliphatic radicals and aromatic radicals, and removing therefrom a zinc concentrate.

3. A method of differential froth flotation which comprises subjecting an aqueous alkaline pulp of an ore containing lead and zinc to froth flotation in the presence of a frother including coal tar creosote in the presence of a reagent included in the group having the following formula:



where  $R_1$  and  $R_3$  are hydrogen atoms and  $R_2$  and  $R_4$  are members chosen from the group including hydrogen, aliphatic radicals and aromatic radicals, said pulp having a pH between 8.0 and 9.0 and being free of any depressing agent for pyrite and sphalerite present in the ore, and removing therefrom a concentrate containing lead and a tailing rich in zinc.

4. A method of differential froth flotation which comprises subjecting an aqueous alkaline pulp of an ore containing lead and zinc to froth flotation in the presence of a frother including coal tar creosote in the presence of a reagent included in the group having the following formula:



where  $R_1$  and  $R_3$  are hydrogen atoms and  $R_2$  and  $R_4$  are members chosen from the group includ-

ing hydrogen, aliphatic radicals and aromatic radicals, said pulp having a pH between 8.0 and 9.0 and being free of any depressing agent for pyrite and sphalerite present in the ore, and removing therefrom a concentrate containing lead, a tailing rich in zinc, activating the zinc with copper sulfate subjecting an aqueous alkaline pulp of the tailing to froth flotation in the presence of a reagent included in the group having the following formula:



15 where  $R_1$  and  $R_3$  are hydrogen atoms and  $R_2$  and  $R_4$  are members chosen from the group including hydrogen, aliphatic radicals and aromatic radicals, said pulp having a pH between 8.0 and 9.0 and being free of any depressing agent for 20 pyrite and sphalerite present in the ore, and removing therefrom a zinc concentrate.

PIERRE R. HINES.

References Cited in the file of this patent

UNITED STATES PATENTS

| Number    | Name       | Date          |
|-----------|------------|---------------|
| 1,208,171 | Lavers     | Dec. 12, 1916 |
| 1,301,551 | Freeman    | Apr. 22, 1919 |
| 1,448,929 | Luckenbach | Mar. 30, 1923 |

OTHER REFERENCES

- Transactions of the American Institute of Mining and Metallurgical Engineers, 1930, pages 301-302. (Copy in Div. 25.)  
 35 Taggart, Handbook of Mineral Dressing, (c) 1945, section 12, page 113. (Copy in Div. 25.)